

J. F. MONNOT.

PROCESS OF MAKING COMPOUND METAL OBJECTS.

APPLICATION FILED JULY 16, 1908.

927,062.

Patented July 6, 1909.

*Fig. 1.*



*Fig. 2.*



*Fig. 3.*



*Fig. 7.*



*Fig. 5.*



*Fig. 4.*



*Fig. 6.*



*Fig. 8.*

Attest:

John F. Monnot

Frank E. Raffman

by

Inventor:  
John F. Monnot  
Marshall & Slocum  
Atty's

# UNITED STATES PATENT OFFICE.

JOHN F. MONNOT, OF NEW YORK, N. Y., ASSIGNOR TO DUPLEX METALS COMPANY, OF NEW YORK, N. Y., A CORPORATION OF NEW YORK.

## PROCESS OF MAKING COMPOUND METAL OBJECTS.

No. 927,062.

Specification of Letters Patent.

Patented July 6, 1909.

Application filed July 16, 1908. Serial No. 443,797.

*To all whom it may concern:*

Be it known that I, JOHN F. MONNOT, a citizen of the United States, residing at New York, in the county of New York and State 5 of New York, have invented certain new and useful Processes of Making Compound Metal Objects, of which the following is a specification.

My invention relates to processes of making compound metal objects and particularly to processes of making objects comprising a core of non-ferrous metal and a coating of ferrous metal, such as steel, such core and coating being weld united.

15 In another application for Letters Patent, Ser. No. 443,796, filed July 16, 1908, I have illustrated and described electrical conductor wire comprising a core of high-conductivity metal, such as copper, and a shell of harder 20 or stronger metal, such as steel, weld united thereto. The present application covers a process of producing such article and other similar articles.

25 In the accompanying drawings I illustrate the method of carrying out my said process and apparatus convenient for use in carrying out the same.

In said drawings: Figure 1 shows a central 30 vertical section of a mold, pouring funnel and an ingot therein formed as hereinafter described. Fig. 2 shows a transverse section of said mold on the line  $z-z$  of Fig. 1. Fig. 3 shows a transverse section of a completed ingot. Fig. 4 shows on a smaller scale, a 35 transverse section of a mold and contents, such as shown in Fig. 1, but including a core by means of which hollow ingots may be produced, and Fig. 5 shows a transverse section of a completed hollow ingot. Fig. 6 shows a top view of a mold adapted for forming 40 rectangular ingots comprising laminæ of ferrous and non-ferrous metals. Fig. 7 shows a vertical section of such mold and of the ingot within it, and Fig. 8 shows a transverse 45 section of a completed ingot.

Referring first to Figs. 1 and 2, 1 designates a circular two-part mold provided with cooling means 2, which in the instance shown is a jacket through which cooling 50 water, oil, etc., is circulated; or compressed air or other suitable gas may be expanded in the jacket space for the purpose of absorbing heat. In the construction shown this mold is assumed to be of metal, iron molds being 55 permissible in casting copper and like metals

against a steel shell or between a steel shell and the sides of the mold, according to the method referred to. But, in lieu of circulation of the cooling fluid through a cooling jacket, as shown, water or other cooling fluid may be played against the outside of the mold, or a mold of very thick metal will, in many cases, in itself have sufficient heat-storage capacity for the purpose desired. Instead of employing a metal mold, a mold 60 of refractory material, for example, a mold of homogenized carbon, such as illustrated and described in my application Sr. No. 430,097 may be used. I have indicated a sectional mold instead of a one piece mold 65 such as commonly used in casting ingots, simply because it is desirable in many cases that the ingot produced shall have no draft vertically; otherwise a one piece mold would be used. The sectional mold comprises suitable means, as for example, bands 3 and wedges 4, to prevent separation of the sections of the mold during the casting, and until the cast metal has solidified.

5 designates a shell or tube of steel or iron 80 to form the steel coating of the resulting article, its thickness being properly proportioned, with reference to the diameter of the ingot, so that this steel shell when extended or drawn down to final size in forming a finished article, will have the desired thickness. This steel shell, before it is placed in the ingot mold, may have been thinly coated by dipping it for a brief interval in supermolten 85 copper or other suitable supermolten coating metal, according to the method set forth in my Patent No. 853,716, in which patent I have set forth a process of producing clad metals based on the fact that while copper and like metals do not form any weld-union 90 when contacted at ordinary casting temperatures with a clean steel surface, yet such a weld union is formed when the copper or like metal with which the steel is contacted is heated to a considerably higher tempera- 95 ture, termed by me in said patent, for the sake of a name, the "supermolten tempera- 100 ture". And as set forth in said patent, a steel object immersed momentarily in a bath of such supermolten unlike metal and then 105 withdrawn under conditions precluding oxidation, will be found covered with a thin welded-on coating of metal of the supermolten bath, and with this coating copper and many other metals when cast there- 110

against at ordinary casting temperatures or slightly higher temperatures, will unite readily and inseparably. Or, the steel shell 5 may have had its surface treated with a vapor of zinc or like metal as set forth in the application of W. M. Page, Ser. No. 443,339, filed July 13, 1908, so producing a surface with which molten copper and like metals at ordinary casting temperatures will unite readily and inseparably; or, the said steel shell may have been heated to a very high white heat before it is placed in the mold so that the molten metal cast within or within and around said shell will be raised, in the immediate vicinity of said shell, to the supermolten condition. Or, as an alternative to the above methods, the copper or like metal may be cast within, or within and around, such shell, while in the supermolten condition.

6 designates a suitable pouring tile or funnel, which may be of refractory material, such as fire clay, or carbon, or may be of metal. In the particular instance shown the shell 5 is of somewhat smaller diameter than the interior diameter of the mold, in order that molten metal may be cast without as well as within said shell and therefore the pouring tile 6 is provided not only with a central space 7 for the introduction of the molten metal for the core, but also with side spaces 8 for the introduction between the shell 5 and the mold of molten coating metal.

35 The metal cast within or within and around the shell 5, is preferably cast through a deep layer of molten wiping material 9, according to the methods set forth in my application Ser. No. 391,674 and my application Ser. No. 443,298, filed July 13, 1908. Such molten wiping material removes oxid impurities and occluded and entrained gases and insures a particularly dense, tough and homogeneous casting, free from blow holes, blebs, etc.; also if this wiping material contains a considerable proportion of oxid-disolving ingredient the mold need be only partly filled with this wiping material prior to the introduction of the molten metal, the molten metal flowing down through this wiping material as it is cast and so displacing upward the wiping material, which is of less specific gravity, said wiping material as it rises, progressively freeing the surface of the shell 5 and, when metal is cast between said shell and the sides of the mold, also freeing the mold walls, of oxid or like impurities, absorbed gases, etc. A suitable wiping material is borax or a mixture of borax and sodium or potassium silicate to which a little fluor spar may be added. The proportions of the ingredients of the wiping material may be varied as required to produce a material which will be freely liquid at the temperature at which the molten metal is cast.

This wiping material may, if desired, be placed in the mold solid, since the first of the molten metal introduced into the mold will melt it; or if the shell 5 be placed at a white heat in the mold, the heat from this shell will suffice in general to melt solid wiping material placed within the mold.

The shell 5 and the wiping material having been placed in the mold as specified, molten copper or other metal to form the core and, if an outer coating is desired, to form such outer coating, is poured into the mold and in passing through the molten wiping material is cleansed as above described, and caused to contact with the surface of the shell 5, and is permitted to solidify against such surface, thereby welding to said surface. Commonly the molten metal will be cast in such quantities as not only to completely fill the mold but also to rise somewhat into the passage or passages of the pouring funnel 6, and owing to the covering of molten wiping material, which material is of low heat conduct capacity, and to the refractory nature of funnel 6 when said funnel is of carbon, clay etc., there will be a head of molten metal within this funnel which will be relatively slow to solidify, and so will fill in any spaces left by contraction of the metal below, the hydrostatic pressure due to this additional height of molten metal and of the wiping material above it further tending to insure a tough dense cast metal free from blow holes and the like. If desired, the molten metal cast between the shell 5 and the walls of the mold, may be cast after the casting of the metal within said shell, after such metal within the shell has begun to solidify, the shrinkage of the metal so cast outside of the shell tending to force the contraction of the shell to keep pace with the contraction of the metal cast within it, and such contraction may be hastened by the circulation of cooling fluid through the jacket 2, the rapid cooling so produced also improving the quality of the cast metal, if it be copper or like metal, and preventing any attack of the metal of the mold, if the mold be of metal, by the cast metal, if the latter be cast at supermolten temperature; and this rapid cooling further tends to prevent attack of the metal of the shell by the cast metal, if the latter be cast at supermolten temperature, to such extent as to contaminate the cast metal. The ingot so produced may be worked in the ordinary manner, either immediately after solidification, or after submission to a soaking heating, and may be rolled and drawn down to final size and shape in the ordinary manner.

Fig. 3 shows a transverse section of a three-layer ingot as removed from the mold, and also in substance shows a cross section of a round object rolled or drawn down from an ingot such as described, since the metals extend substantially in the same proportion,

preserving the same relative thickness when weld united. In Fig. 3, 10 designates a core of copper or like non-ferrous metal, 11 a coating of steel and an outer coating of copper 12 or like metal. This outer coating may be of any thickness desired. It may be very much thicker relatively than as shown in Fig. 3, or it may be very much thinner. Where the core and outer layer are relatively thick, the intermediate layer of steel serves mainly as a mechanical reinforcement, giving, because of its tubular form, more strength for the same amount of steel than would a central steel core. It is not necessarily the same metal as that of core 10. In most cases the principal function of this outer coating 12 will be to protect the steel coating 11 from oxidation or like chemical attack; therefore it may be very thin. But in many cases the outer coating 12 of non-ferrous metal may be omitted altogether. Likewise the steel tube or separator 5 may have any desired thickness with reference to the thickness of the core and of the outer coating 12, if an outer coating be provided. It may be even thicker, relatively, than indicated in the drawing, or may be very much thicker. Particularly in the case of hollow ingots such as illustrated in Fig. 5, which shows a coated and lined steel shell 5 the thickness of the steel shell may be very much greater than that of either coating cast against it. Ingots so produced may be used in the manufacture of seamless tubing by the Mannesmann or other tube-forming process, including the ordinary methods of tube drawing.

In Fig. 4 I have shown a mold 1 such as shown in Fig. 1, and a steel tube 5 within said mold and within said tube, a collapsible core 13 leaving a space between it and the inner surface of the shell 5 into which molten metal may be cast. A space between the outer surface of the shell and the inner surface of the mold, into which metal may be cast, may or may not be provided, as preferred.

The same process may also be used for forming ingots comprising laminæ of ferrous and non-ferrous metals alternated. Figs. 6 and 7 illustrate a mold adapted for such purpose and Fig. 8 shows a cross section of the completed ingot. The mold, 14, is of sectional construction, though this is not material, as previously explained; and in the mold are inserted a suitable number of ferrous metal separators 15, the non-ferrous metal or metals being poured around these separators. These separators may have any desired thickness with reference to the thickness of the layers of non-ferrous metal; i. e., may either be very thin, relatively or very thick, relatively.

For convenience in heating the molds, before the introduction of the molten metal, I

commonly provide in the bottom of the mold, whether of the form shown in Fig. 1 or of the form shown in Figs. 6 and 7, an opening through which the flame from a suitable burner may be projected into the mold, such opening being closed, before the introduction of molten metal, by a plug 16 of such material as is commonly used in closing the tap holes of cupolas, or any other suitable material.

7.5

What I claim is:—

1. A process of producing compound metal objects comprising unlike metals weld united, which comprises casting molten bodies of non-ferrous metal into contact with opposite surfaces of a separator of ferrous metal under conditions of temperature of molten metal, or separator, or both, adapted for forming a weld union, and permitting the molten metal so cast to solidify as soon as such weld union is effected.

2. A process of producing compound metal objects comprising unlike metals weld united, which comprises casting molten bodies of non-ferrous metal into contact with opposite surfaces of a separator of ferrous metal under conditions of temperature of molten metal, or separator, or both, adapted for forming a weld union, progressively cleaning one or both said surfaces by the action thereon of a deep layer of molten flux containing oxid-dissolving material and permitting the molten metal so cast to solidify.

3. A process of producing compound metal objects comprising a ferrous metal annulus and a layer of non-ferrous metal within said annulus and weld-united thereto, which comprises casting molten non-ferrous metal within a tube or shell of ferrous metal and in contact with the inner surface thereof, under conditions of temperature of the molten metal, or tube, or both, adapted for forming a weld union, and permitting the molten metal so cast to solidify as soon as such weld union is effected.

4. A process of producing compound metal objects comprising a ferrous metal annulus and a layer of non-ferrous metal within said annulus and weld-united thereto, which comprises casting molten non-ferrous metal within a tube or shell of ferrous metal and in contact with the inner surface thereof, under conditions of temperature of the molten metal, or tube, or both, adapted for forming a weld union, progressively cleaning one or both said surfaces by the action thereon of a deep layer of molten flux containing oxid-dissolving material and permitting the molten metal so cast to solidify.

5. A process of producing compound metal objects comprising unlike metals weld united, which comprises casting molten bodies of copper into contact with opposite surfaces of a separator of steel under conditions of temperature of molten metal, or separator, or

125

115

120

125

130

both, adapted for forming a weld union, and permitting the molten metal so cast to solidify as soon as such weld union is effected.

6. A process of producing compound metal objects comprising unlike metals weld united, which comprises casting molten bodies of copper into contact with opposite surfaces of a separator of steel under conditions of temperature of molten metal, or separator, or both, adapted for forming a weld union, progressively cleaning one or both said surfaces by the action thereon of a deep layer of molten flux containing oxid-dissolving material and permitting the molten metal so cast to solidify.

7. A process of producing compound metal objects comprising a steel annulus and a layer of copper within said annulus and weld-united thereto, which comprises casting molten copper within a tube or shell of steel and in contact with the inner surface thereof, under conditions of temperature of the molten metal, or tube, or both, adapted for form-

ing a weld union, and permitting the molten metal so cast to solidify as soon as such weld union is effected.

8. A process of producing compound metal objects comprising a steel annulus and a layer of copper within said annulus and weld-united thereto, which comprises casting molten copper within a tube or shell of steel and in contact with the inner surface thereof, under conditions of temperature of the molten metal, or tube, or both, adapted for forming a weld union, progressively cleaning one or both said surfaces by the action thereon of a deep layer of molten flux containing oxid-dissolving material and permitting the molten metal so cast to solidify.

In testimony whereof I affix my signature, in the presence of two witnesses.

JOHN F. MONNOT.

Witnesses:

H. M. MARBLE,  
FRANK E. RAFFMAN.